

# United States Patent Office

3,556,873

Patented Jan. 19, 1971

1

3,556,873

## SILICON STEELS CONTAINING SELENIUM

Frank A. Malagari, Jr., Freeport, Pa., assignor to Allegheny Ludlum Steel Corporation, Brackenridge, Pa., a corporation of Pennsylvania  
No Drawing. Filed Apr. 12, 1968, Ser. No. 721,099  
Int. Cl. H01f 11/16; C22c 39/46, 39/54  
U.S. Cl. 148—31.55

4 Claims

### ABSTRACT OF THE DISCLOSURE

Described is grain oriented silicon steel having a predominantly (110) [001] texture and critical carbon, manganese and selenium quantities, i.e., 0.02% to 0.07% carbon, at least 0.045% manganese, 0.01% to 0.1% selenium and not more than residual sulfur.

This invention relates to grain oriented silicon steel. More particularly, the invention concerns silicon steel containing critically controlled quantities of carbon, manganese and selenium and having a predominantly (110) [001] texture.

Recently, the addition of selenium to silicon steels has received considerable attention as a technique for achieving preferred orientation in these compositions; however, the addition of selenium does not necessarily improve the properties of such steels.

In accordance with the invention, it has been discovered that selenium can be made to exercise a beneficial effect on the properties of silicon steel having not more than residual sulfur, if the carbon, manganese and selenium are critically controlled. As is hereinafter described, manganese must be present in a carefully defined range for selenium to be beneficial for good texture development. While the phenomenon involved is not entirely

2

0.045% to 0.07% manganese, not more than residual sulfur, i.e., less than 0.008%, 0.01% to 0.1% selenium, preferably 0.02% to 0.08% selenium, and having a predominantly (110) [001] texture. Optimum properties of core loss and permeability are obtained by compositions having the nominal analysis 0.05% carbon, 0.06% manganese, 3.4% silicon, 0.04% selenium, 0.002% sulfur and 0.004% phosphorus, the balance essentially iron and other steel-making residuals. This composition has a 60 cycle core loss of 0.44 watt per pound at 15,000 gauss and a permeability at 10 oersteds of 1845.

The following examples will illustrate grain oriented silicon steels in accordance with the invention and the improved properties which they possess.

15 A series of samples of the compositions described in Table I were prepared by vacuum induction melting, hot rolled from ingot to band gauge, normalized, cold rolled to intermediate gauge, normalized and cold rolled to final gauge. After final cold rolling, the strip was given a 20 decarburizing anneal.

TABLE I

| Group | Master alloy | C    | Mn   | P    | S    | Si   | Se     |
|-------|--------------|------|------|------|------|------|--------|
| I     | RV-2184      | .030 | .060 | .004 | .003 | 3.33 | 0-.14  |
| II    | RV-2185      | .053 | .060 | .004 | .002 | 3.38 | 0-.13  |
| III   | RV-2203      | .034 | .008 | .007 | .020 | 3.25 | 0-.09  |
| IV    | RV-2183      | .054 | .008 | .008 | .020 | 3.33 | 0-.096 |

Specifically, each of the compositions described in Table I were hot rolled from 2400° F. to hot band gauge ranging in thickness from 0.077 to 0.083 inch. The sample material was heat treated for 30 minutes at 1830° F., cold rolled to the intermediate gauge of 0.028 inch and normalized at 1725° F. Thereafter, the samples were then cold rolled to 0.0108 inch and given a final normalizing at 1475° F. after which they were then given a texture anneal with a maximum temperature of 2150° F. for purification. The magnetic properties are described in Table II.

TABLE II

| Group | Heat   | Percent Se | Percent Mn | Percent S | Percent C | 60~WPP at 15 kb. | 60~m <sub>u</sub> at 10 h. |
|-------|--------|------------|------------|-----------|-----------|------------------|----------------------------|
| I     | 2C1162 | 0          | .060       | .003      | .030      | *.559 (.586)     | *1,678 (1,668)             |
|       | 2C1147 | .01        | .060       | .003      | .030      | .512 (.554)      | 1,735 (1,693)              |
|       | 2C1148 | .02        | .060       | .003      | .030      | .530 (.555)      | 1,740 (1,701)              |
|       | 2C1149 | .04        | .060       | .003      | .030      | .512 (.510)      | 1,750 (1,786)              |
|       | 2C1150 | .06        | .060       | .003      | .030      | .482 (.485)      | 1,821 (1,816)              |
|       | 2C1151 | .08        | .060       | .003      | .030      | .460 (.481)      | 1,826 (1,819)              |
|       | 2C1152 | .14        | .060       | .003      | .030      | .575 (.554)      | 1,743 (1,771)              |
| II    | 2C1139 | 0          | .060       | .002      | .053      | .551 (.552)      | 1,692 (1,703)              |
|       | 2C1140 | .01        | .060       | .002      | .053      | .483 (.516)      | 1,762 (1,766)              |
|       | 2C1141 | .02        | .060       | .002      | .053      | .454 (.459)      | 1,806 (1,831)              |
|       | 2C1142 | .04        | .060       | .002      | .053      | .440 (.451)      | 1,845 (1,827)              |
|       | 2C1143 | .06        | .060       | .002      | .053      | .477 (.490)      | 1,819 (1,802)              |
|       | 2C1144 | .08        | .060       | .002      | .053      | .484 (.525)      | 1,810 (1,805)              |
|       | 2C1145 | .13        | .060       | .002      | .053      | .548 (.566)      | 1,755 (1,755)              |
| III   | 2C1133 | 0          | .008       | .020      | .034      | .783             | 1565                       |
|       | 2C1134 | .01        | .008       | .020      | .034      | .681             | 1615                       |
|       | 2C1135 | .02        | .008       | .020      | .034      | .718             | 1611                       |
|       | 2C1136 | .04        | .008       | .020      | .034      | .794             | 1600                       |
|       | 2C1137 | .06        | .008       | .020      | .034      | .840             | 1558                       |
|       | 2C1138 | .09        | .008       | .020      | .034      | .681             | 1648                       |
| IV    | 2C1126 | 0          | .008       | .020      | .054      | .544             | 1729                       |
|       | 2C1127 | .01        | .008       | .020      | .054      | .592             | 1677                       |
|       | 2C1128 | .02        | .008       | .020      | .054      | .516             | 1747                       |
|       | 2C1129 | .04        | .008       | .020      | .054      | .914             | 1504                       |
|       | 2C1130 | .06        | .008       | .020      | .054      | .732             | 1611                       |
|       | 2C1131 | .08        | .008       | .020      | .054      | .558             | 1727                       |
|       | 2C1132 | .096       | .008       | .020      | .054      | .586             | 1705                       |

\*Data in parenthesis on a second series of samples of the same composition.

understood, it is believed to involve the formation of manganese selenide which is in turn responsible for the improved properties.

Grain oriented silicon steels within the purview of the invention are those containing 0.02% to 0.07% carbon, 2% to 4% silicon, at least 0.045% manganese, preferably

70 It is evident from the data in Table II that low core loss with high permeability occurs in the 0.03% carbon series (Group I) at selenium contents of 0.06% and 0.08%. This group of samples also has a sulfur content in the residual range but the manganese content is 0.06%. Below or above this selenium range the core loss is higher with a corre-

sponding decrease in permeability. However, if the carbon level is increased to 0.053%, as in the Group II

higher silicon content detrimentally affects the cold workability of the steel.

TABLE III

| Aim Se, percent | Series No. 1            |                   |                 | Series No. 2            |                   |                | Sulfur Series           |                   |  |
|-----------------|-------------------------|-------------------|-----------------|-------------------------|-------------------|----------------|-------------------------|-------------------|--|
|                 | 60~<br>WPP at<br>15 kb. | $\mu$ at<br>10 h. | Aim Se, percent | 60~<br>WPP at<br>15 kb. | $\mu$ at<br>10 h. | Aim S, percent | 60~<br>WPP at<br>15 kb. | $\mu$ at<br>10 h. |  |
| 0.....          | .551                    | 1,692             | 0               | .561                    | 1,694             | .....          | .....                   | .....             |  |
|                 | .552                    | 1,687             |                 |                         |                   |                |                         |                   |  |
| .01.....        | .483                    | 1,762             | .01             | .527                    | 1,709             | .01            | .618                    | 1,689             |  |
|                 | .505                    | 1,745             |                 |                         |                   |                |                         |                   |  |
| .02.....        | .454                    | 1,806             | .02             | .483                    | 1,793             | .02            | .520                    | 1,784             |  |
|                 | .465                    | 1,818             |                 |                         |                   |                |                         |                   |  |
| .04.....        | .440                    | 1,845             | .04             | .469                    | 1,803             | .03            | .558                    | 1,774             |  |
|                 | .478                    | 1,810             |                 |                         |                   |                |                         |                   |  |
| .06.....        | .477                    | 1,819             | .06             | .463                    | 1,856             |                |                         |                   |  |
|                 | .473                    | 1,812             |                 |                         |                   |                |                         |                   |  |
| .08.....        | .484                    | 1,810             | .08             | .513                    | 1,809             | .07            | .687                    | 1,623             |  |
|                 |                         |                   |                 |                         |                   |                |                         |                   |  |
| .13.....        | .548                    | 1,755             |                 |                         |                   |                |                         |                   |  |
|                 | .571                    | 1,731             |                 |                         |                   |                |                         |                   |  |

samples, then the best core loss and permeability combination occurs at 0.02% and 0.04% selenium. Thus, it is possible to obtain excellent core loss at lower selenium levels if the carbon is increased to about the 0.05% level. Continued good core loss and permeability can be obtained with selenium contents of 0.08% and some deterioration in magnetic properties occurs at above about 0.1% selenium. It should be noted that the manganese content for the Group II samples was also about 0.06%.

The test results for the samples in Groups III and IV have higher sulfur, i.e., 0.2%, but very low manganese, i.e., 0.008%, together with selenium. The poor properties shown illustrate the importance of manganese control and that selenium is not beneficial in sulfur-containing steels. It has been determined that manganese levels below about 0.045% will not result in consistently satisfactory properties.

It has also been found that optimum properties in silicon steels in accordance with the invention are achieved at selenium levels of 0.02% to 0.08%. This is seen by the series of examples summarized in Table III which compares the electrical properties of selenium-containing steels with those of sulfur-containing steels. It is evident from the data in Table III that extremely low core losses can be obtained in selenium-bearing 3.25% silicon steels. It has also been determined by comparison with sulfur-bearing steels that silicon would have to be increased to about 4% to achieve a comparable core loss level in sulfur-containing steels devoid of selenium. Of course,

The improved electrical properties in the silicon steel disclosed above and in the foregoing examples reflect the strong development of the (110) [001] texture. The development of this texture results in extremely low core loss with high permeability. Properties of the steels in accordance with the invention can be optimized by controlling the carbon content within the range of 0.03% to 0.053%.

It is apparent from the above that various changes and modifications may be made without departing from the invention. Accordingly, the scope of the invention should be limited only by the appended claims.

I claim:

1. Grain oriented silicon steel having a predominantly (110) [001] texture consisting essentially of 0.02% to 0.07% carbon, 2% to 4% silicon, at least 0.045% manganese, 0.01% to 0.1% selenium and less than about 0.008% sulphur.

2. Grain oriented silicon steel in accordance with claim 1 having 0.02% to 0.8% selenium.

3. Grain oriented silicon steel in accordance with claim 1 consisting essentially of 0.02% to 0.07% carbon, 2% to 4% silicon, 0.045% to 0.07% manganese, 0.02% to 0.08% selenium and not more than 0.008% sulphur.

4. Grain oriented silicon steel in accordance with claim 3 having, normally, 0.05% carbon, 0.06% manganese, 3.4% silicon and 0.04% selenium.

#### References Cited

#### UNITED STATES PATENTS

- 2,867,557 1/1959 Crede et al. ----- 148—111  
 3,151,005 9/1964 Alworth et al. ----- 148—113  
 3,157,538 11/1964 Imai et al. ----- 148—110X

L. DEWAYNE RUTLEDGE, Primary Examiner

G. K. WHITE, Assistant Examiner

U.S. Cl. X.R.

75—123; 148—111, 112